

Feb. 25, 1947.

L. G. SELMI ET AL

2,416,648

ALLOY STEEL

Filed March 4, 1942

4 Sheets-Sheet 1



FIG. I.

BY

INVENTOR  
LUCIANO G. SELMI and  
CLARENCE L. ALTBURGER

*Gay, MacLean, Gobrick  
Williams, Hilton and Adler*  
ATTORNEYS.

Feb. 25, 1947.

L. G. SELMI ET AL

2,416,648

ALLOY STEEL

Filed March 4, 1942

4 Sheets-Sheet 2



FIG.2.

BY

INVENTOR.  
LUCIANO G. SELMI and  
CLARENCE L. ALtenburger  
*Fay Macklin Golub*  
*Williams, Hilton and Dene*  
ATTORNEYS.

Feb. 25, 1947.

L. G. SELMI ET AL

2,416,648

ALLOY STEEL

Filed March 4, 1942

4 Sheets-Sheet 3



CASE CARBURIZED 8 HRS AT 1700°F

|    |      |    |     |
|----|------|----|-----|
| C  | .18  | Si | .84 |
| Mn | .78  | Cr | .60 |
| P  | .019 | Mo | .15 |
| S  | .019 | Zr | .13 |

INVENTORS

LUCIANO G. SELMI and  
CLARENCE L. ALTBURGER

Fay Macklin Goldrich  
Williams, Keltin and Goldrich  
ATTORNEYS

FIG. 3.

Feb. 25, 1947.

L. G. SELMI ET AL

2,416,648

## ALLOY STEEL

Filed March 4, 1942

4 Sheets-Sheet 4



FIG. 4

*INVENTORS.*

LUCIANO G. SELMI and  
CLARENCE L. ALTEMBERGER.

BY

Fay Macklin & Schuch  
Williams, Chilton and Isler.  
ATTORNEYS

## UNITED STATES PATENT OFFICE

2,416,648

## ALLOY STEEL

Luciano G. Selmi, Detroit, and Clarence L. Altenburger, Dearborn, Mich., assignors to Great Lakes Steel Corporation, Ecorse, Mich., a corporation of Delaware

Application March 4, 1942, Serial No. 433,384

## 1. Claim. (Cl. 148—31)

1

This invention relates to improvements in low alloy, high tensile steels which are adapted to be heat treated.

Examples of such steels have been described in our United States Patents Nos. 2,234,130, now Reissue No. 22,072, and 2,250,505, and our co-pending application, Serial No. 403,188, filed July 19, 1941.

In the steels described in said patents and co-pending application, the amounts of alloying elements are within narrow ranges, although comparatively wide variations in the amounts of carbon and molybdenum are given.

Objects of the present invention are to provide:

- (1) A fine grained steel;
- (2) Stable against strain aging; and
- (3) Especially suited in thinner gauges where molybdenum contributes too much hardness to "as rolled" or "normalized" steel.

The application, Serial No. 403,188 and the re-issue patent above mentioned, teaches varying the molybdenum content. The application gives hardness tables of steels designated, "X—Y—Z" showing varying silicon and manganese, and following these tables we speak of varying the manganese content up to 1.00%. According to our present discovery there is a definite relationship for a most effective and economical use of molybdenum in amounts having a relation to the other elements, particularly manganese as hereinafter appears.

The general increasing desire and demands for substitutions of low alloys for even wider uses than heretofore contemplated have prompted further investigation and researches for steels of the nature of those set forth in our above identified patents and we have found we may attain additional desirable characteristics and improved particularly hardenability values in relation to molybdenum and other alloy contents.

The present application teaches specifically the provision of a widely useful steel in which alloying elements of great importance in the war program, such as chromium, silicon, manganese and molybdenum, are used in minimum quantities.

By the present invention we may use molybdenum more effectively and economically. We attain exceptional hardenability or depth hardening capacity and adaptability for case carburizing, giving a case structure showing a virtual lack of cementitic membranes.

In our first mentioned patent is described an analysis with low molybdenum content and which was capable of hardening in thin sections but was not fully satisfactory for heavier sections.

A special object of the present invention is the provision of a low alloy steel having a maximum hardenability relative to the amount of each element and to the total of its contained alloys.

2

The size of section in which this maximum hardness, or some other lower hardness which might arbitrarily be selected, may be attained throughout, depends upon "hardenability" which is a function and an effect of the amounts, nature and ratios of varying alloying elements.

This application is particularly concerned with our discovery that in an alloy of this type a certain proportionate amount of molybdenum added for heat treating purposes has a critical upper limit and practical lower limit. More molybdenum may increase the overall hardness of the alloy as rolled or slow cooled but it does not advantageously increase the hardenability or depth hardening characteristics obtained in heat treating.

For convenient illustration and comparison of the effects of modification of chemistry, physical properties and characteristics, reference may be had to the accompanying drawings in which:

Fig. 1 is a chart showing the heat treating characteristics of specific examples of the alloy of the present invention having varying proportions of molybdenum, and

Fig. 2 is a chart diagrammatically illustrating the rate of change of hardness of the alloy with increasing amounts of molybdenum.

Fig. 3 is a microphotograph showing the structure of such a steel, magnification being approximately 100 $\times$  and taken of a sample having the chemical alloying elements tabulated below this figure.

Fig. 4 is a chart showing physical properties.

Referring more particularly to Fig. 1, it will be apparent that with increasing amounts of molybdenum, the hardenability of the alloy increases proportionally up to about .15% molybdenum, after which the increase in hardenability for added increases of molybdenum falls off rapidly. The curve of Fig. 2 was plotted from values representing the curvature of the curves at the depth of twenty-sixteenths, as shown and these values were determined in the manner described on pages 76 and 77 Love's Differential and Integral Calculus published in 1918.

It will be apparent from an inspection of Fig. 2 that the optimum needed percentage of molybdenum is about .15% in the low carbon ranges herein given. In practice, however, due to the presence of varying amounts of molybdenum in the scrap used and other factors beyond the control of the operator, it is impractical to come closer than about .05% either side of the desired proportion. Since, as shown in Fig. 2, the hardenability changes very rapidly below .10% molybdenum, a proportion finally arrived at in the finished steel with a content appreciably below .10% would result in a very much decreased hardenability. On the other hand, since the curve of Fig. 2 is relatively flat between .10%

and .20% molybdenum, it is advisable to arrive at a finished steel having a molybdenum content within this range. With over .20% molybdenum it is apparent that there is little change in hardenability. Thus we find a critical upper limit to the amount which would be used where the heat treating characteristics of the steel are controlling within the limits given in the examples for the amounts of other elements, particularly manganese. The lower practical limit of .10% and the upper critical limit of .20% molybdenum would normally, in practice, teach an addition of molybdenum such as to arrive at .15% in the finished steel. Conditions beyond the control of the steel maker would normally vary the resulting proportion of molybdenum in the finished steel somewhere between .10% and .20%.

With manganese .75% to .80% any increase in

A steel of this specific analysis is especially desirable where objects difficult to cold form are to be made and heat treated to definite physical properties. The hardenability of the steel, as to plain end quench bars, is substantially the same as that of steels comprised within the series SAE-4415 to SAE-4620.

Improved values of tensile strength, yield point, Izod impact values, reduction in area and elongation of an example of our steel, containing .16% carbon, .74% manganese, .85% silicon, .59% chromium, .15% molybdenum, .16% zirconium, .018% sulphur, and .029% phosphorus are attained, were shown in Fig. 1 of our Patent No. 2,234,130. Compare the values on Chart Fig. 4 noting the molybdenum .15%.

The hardenability of examples of steels of the present invention is indicated in the table below:

HARDENABILITY TABLE  
PLAIN END QUENCH BAR TEST  
1" DIAMETER X 3" LONG  
Rockwell "C" hardness

| Distance, 16ths       | X-15  |       |       | X-20  |       |       | X-25  |       |       | Fine  |
|-----------------------|-------|-------|-------|-------|-------|-------|-------|-------|-------|-------|
|                       | X-15  | X-20  | X-25  | X-15  | X-20  | X-25  | X-15  | X-20  | X-25  |       |
| 1                     | 41    | 42    | 44    | 46    | 47    | 47    | 47    | 47    | 48    | 46    |
| 2                     | 40    | 40    | 44    | 45    | 46    | 46    | 47    | 47    | 48    | 46    |
| 3                     | 36    | 37    | 42    | 43    | 42    | 42    | 47    | 47    | 48    | 45    |
| 4                     | 33    | 31    | 37    | 39    | 38    | 38    | 42    | 45    | 47    | 44    |
| 5                     |       |       | 33    | 35    | 33    | 36    |       | 43    | 43    | 41    |
| 6                     | 29    | 25    | 30    | 32    | 30    | 32    |       | 40    | 40    | 38    |
| 7                     |       |       | 28    | 30    | 28    | 31    |       | 37    | 37    | 36    |
| 8                     | 25    | 21    | 26    | 28    | 27    | 29    | 30    | 36    | 36    | 35    |
| 10                    |       |       | 24    | 25    | 25    | 27    |       | 33    | 33    | 31    |
| 12                    | 19    | 14    | 23    | 24    | 22    | 25    | 27    | 31    | 31    | 30    |
| 14                    |       |       | 21    | 22    | 22    | 24    |       | 29    | 30    | 29    |
| 16                    | 17    | 10    | 20    | 21    | 20    | 22    | 22    | 29    | 28    | 27    |
| 20                    | 16    | 8     | 18    | 20    | 20    | 20    | 22    | 26    | 27    | 26    |
| 24                    | 13    | 6     | 15    | 19    | 19    | 20    | 22    | 26    | 27    | 24    |
| 28                    | 12    | 6     | 12    | 18    | 17    | 20    | 22    | 26    | 24    | 25    |
| 32                    | 10    | 5     | 10    | 17    | 17    | 18    | 25    | 25    | 24    | 25    |
| Grain size            | Fine  | Fine  | Fine  | Fine  | Fine  | Fine  | Fine  | Fine  | Fine  | Fine  |
| Quench temp., deg. F. | 1,630 | 1,630 | 1,630 | 1,700 | 1,700 | 1,700 | 1,700 | 1,600 | 1,700 | 1,625 |
| C                     | .15   | .16   | .19   | .19   | .22   | .22   | .23   | .24   | .23   | .23   |
| Mn                    | .74   | .68   | .77   | .72   | .67   | .61   | .79   | .81   | .75   | .75   |
| P                     | .029  | .030  | .019  | .021  | .018  | .012  | .013  | .026  | .021  | .018  |
| S                     | .018  | .023  | .019  | .018  | .020  | .018  | .015  | .020  | .018  | .018  |
| Si                    | .85   | .80   | .90   | .96   | .79   | .63   | .64   | .94   | .99   | .99   |
| Cr                    | .59   | .52   | .60   | .63   | .63   | .62   | .66   | .59   | .64   | .64   |
| Mo                    | .15   | .09   | .08   | .18   | .17   | .21   | .14   | .17   | .15   | .15   |
| Zr                    | .16   | .14   | .13   | .16   | .11   | .11   | .12   | .19   | .17   | .17   |

molybdenum over .15% does not contribute materially to the hardenability of the alloy. However, if the manganese be increased to .85% to .95% a material increase in hardenability is obtained by changing the molybdenum content from .15% to .20%.

The steel of the present invention, in addition to iron and incidental impurities, preferably contains the following elements within the ranges specified:

|            | Per cent |
|------------|----------|
| Carbon     | .06-.24  |
| Manganese  | .30-.75  |
| Silicon    | .60-.90  |
| Chromium   | .30-.75  |
| Molybdenum | .10-.20  |
| Zirconium  | .10-.20  |
| Sulphur    | .05-Max. |
| Phosphorus | .04-Max. |

A typical alloy within the foregoing range will contain:

|            | Per cent |
|------------|----------|
| Carbon     | .16      |
| Manganese  | .69      |
| Silicon    | .85      |
| Chromium   | .51      |
| Molybdenum | .15      |
| Zirconium  | .14      |
| Sulphur    | .023     |
| Phosphorus | .032     |

From the foregoing table, it will be apparent that the hardenability of our steels compare very favorably with known and widely used steels of higher amounts of alloying elements, for example, our steel designated at the top of the column, 50 X-20 compares favorably with well-known higher chrome steel SAE-4120 similarly, our steels listed under the columns headed X-25 may be compared favorably to the high content nickel steels known as SAE-4820 in respect to the 55 hardenability.

It is apparent, by comparison of our present 60 steel with the properties, including the hardenability of standard widely used steels having like properties and characteristics, that marked and important savings of strategic and valuable alloying elements may be effected, while the very 65 desirable objectives of steels having these improved characteristics may be attained without special treatment or equipment.

As previously mentioned the steels are well-adapted for case carburization, the case structure in the hypereutectoid zones showing a virtual lack of cementitic membranes, Fig. 3 showing the micrographic structures of a carburized case of a 70 steel of the analysis indicated.

Steels of the present invention are particularly adapted for manufacture into special articles, such, for example, as oxygen supply cylinders, bombs, airplane wheels, rivets, army helmets, gears, etc.

Likewise, and by reason of the same properties and characteristics attained, steels made according to our present invention are suitable for a wide variety of civilian uses such as automobile and truck gears.

Having thus described our invention, the nature and scope thereof are defined in the appended claim, it being understood that the particular relationships and ranges specified may be subject to slight or reasonable variations without departing from the spirit of our invention.

We claim:

A carburized steel article containing as essential alloying elements about 0.5 to about .75 per cent of chromium, about 0.6 to about 0.9 per cent of silicon, about 0.1 to about 0.2 per cent of molybdenum, .10 to .20 per cent of zirconium, carbon from 0.1 to about 0.24 per cent and in an amount such that the steel is hardenable by heat treatment, and the remainder iron together with

10

20

impurities and elements in amounts which do not adversely affect the carburizing and heat treating characteristics of the steel, and characterized by a carburized case resistant to spalling and low in or substantially free from massive carbides, and high tensile strength in the core as the result of heat treatment.

LUCIANO G. SELMI.  
CLARENCE L. ALTBURGER.

#### REFERENCES CITED

The following references are of record in the file of this patent:

#### UNITED STATES PATENTS

| Number    | Name  | Date          |
|-----------|-------|---------------|
| 1,278,082 | Wills | Sept. 3, 1918 |
| 2,250,505 | Selmi | July 29, 1941 |
| 2,234,130 | Selmi | Mar. 4, 1941  |